

## UNITED STATES PATENT OFFICE

GUSTAV KÖGEL, OF KARLSRUHE, GERMANY

## LIGHT SENSITIVE LAYER AND PROCESS OF PREPARING IT

No Drawing. Application filed December 4, 1928, Serial No. 323,801, and in Germany December 13, 1927.

The present invention relates to the preparation of light-sensitive layers by means of ferric salts.

I have found that light-sensitive layers suitable for copying a positive from a negative can be obtained by means of ferric salts, the process being carried out by mixing the ferric salts with ketones which, when exposed to light, yield color compounds.

For the preparation of the layer there is used as first component a ferric compound, such as ferric ammonium citrate ferric ammonium tartrate, ferric-ammonium oxalate or the like; also ferric chloride and ferric sulfate mixed with each other.

As second component there are used ketones which are capable of combining with ferrous salts so as to form color compounds. Among those compounds quinones are particularly suitable in the new process, for instance beta-naphthoquinonesulfonic acid, nitroso compounds, or isonitroso compounds of beta-carbonyl compounds of an aliphatic, aromatic, or aliphatic-aromatic character.

The above mentioned ferric compounds are reduced to ferrous compounds on exposure to light and form, on being coupled with the second component, directly visible coloring matter.

There may be added to the layer some binding material, such as gelatin or starch; also metallic salts which are suitable for reducing the solubility of the dyestuffs, and any additional mordant. If a silver compound is added to the layer, copies of the type of the so-called "Sepia"—paper are obtained.

By the new process it is possible to obtain pictures which exhibit the greater part of the coloration already during the copying operation, so that the washing—and developing operations only serve to complete the coloration and to remove the surplus of the chemical substances.

The following example serves to illustrate my invention but is not intended to limit it thereto:

A mixture of 1 part of ferric ammonium

citrate with 3 parts of isonitrosoacetylacetone and some hydrolyzed starch and barium chloride added thereto is applied on paper. After the layer has been dried, it is exposed to light under a pattern. The picture is immediately produced whereupon it is treated with water. In the same manner may be used isonitrosopropionylacetone, also nitroso-beta-naphthol or the like. When using beta-naphtholquinone-4-sulfonic acid, pictures with a more greenish tone are obtained.

If the pictures require to be mordanted subsequently, this can be done by means of a bichromate or the like.

I claim:

1. The process of preparing light-sensitive layers, suitable for taking a positive from a negative, by means of a ferric salt, which process consists in combining a ferric salt with a compound of the following formula:



wherein X stands for alkyl.

2. The process of preparing light-sensitive layers, suitable for taking a positive from a negative, by means of ferric ammonium citrate, which process consists in combining said ferric ammonium citrate with a compound of the following formula:



3. Light-sensitive layers, suitable for taking a positive from a negative, which consist of a ferric salt and a compound of the following formula:



wherein X stands for alkyl.

4. Light-sensitive layers, suitable for taking a positive from a negative, which consist of a ferric ammonium citrate and a compound of the following formula:



5. The process of preparing light-sensitive layers, suitable for taking a positive from

a negative, by means of a ferric salt, which process consists in combining a ferric salt with a compound selected from the group consisting of beta-naphthoquinone-sulfonic acid, isonitrosoacetyl-acetone, isonitrosopropionyl-acetone and nitroso-beta-naphthol.

6. The process of preparing light-sensitive layers, suitable for taking a positive from a negative, by means of ferric ammonium citrate, which process consists in combining said ferric ammonium citrate with a compound selected from the group consisting of beta-naphthoquinone-sulfonic acid, isonitrosoacetyl-acetone, isonitrosopropionyl-acetone and nitroso-beta-naphthol.

7. Light-sensitive layers, suitable for taking a positive from a negative, which consist of a ferric salt and a compound selected from the group consisting of beta-naphthoquinone-sulfonic acid, isonitrosoacetyl-acetone, isonitrosopropionyl-acetone and nitroso-beta-naphthol.

8. Light-sensitive layers, suitable for taking a positive from a negative, which consist of a ferric ammonium citrate and a compound selected from the group consisting of beta-naphthoquinone-sulfonic acid, isonitrosoacetyl-acetone, isonitrosopropionyl-acetone and nitroso-beta-naphthol.

28 In testimony whereof, I affix my signature.  
GUSTAV KÖGEL.

35

40

45

50

55

60

65